

## UNITED STATES PATENT OFFICE

2,139,939

## METHOD OF PRODUCING AN IRON ALLOY

William J. Doyle and Justus J. Wollenhaupt, Cincinnati, Ohio, assignors of one-half to The Williamson Heater Company, Cincinnati, Ohio, a corporation of Ohio, and one-half to Sears, Roebuck and Co., Chicago, Ill., a corporation of New York

No Drawing. Application May 15, 1936,  
Serial No. 79,922

3 Claims. (Cl. 75—126)

This invention relates to the production of a cast-iron alloy of such nature that when used to form objects that are subjected to frequent and considerable heat such objects will not substantially and permanently increase in size, change in shape or undergo undue cracking from repeated heating. An illustration of some of such objects are those parts of a cast-iron warm air furnace, stove or the like, that are subjected to the direct and repeated actions of the heat such as the firepots, fire domes, grates and the like. These examples are to be understood as illustrative only and not as limiting the scope of our invention, as many other illustrations might be cited as being equally applicable.

It has been the history of cast-iron warm air furnaces and stoves, that certain parts will frequently crack or burn out when operating under certain unfavorable conditions such as over-firing of the furnace, the use of certain types of coal, insufficient air supply to the heater, and other conditions. The need has long been felt of being able to develop some kind of cast-iron which would have properties that would more greatly resist and minimize these conditions.

Upon high heating, prior to the present invention, the castings subjected to the direct and repeated actions of the heat would expand, and when allowed to cool would contract. This repeated expansion and contraction has a wearing and tearing action upon the fibre of the cast-iron. Under each reheating they would expand more and more and never eventually return to their original or true dimensions. They would generally warp out of shape irregularly and unevenly. In doing this they would frequently carry this warpage into adjoining castings which are fitted to them. Damage is thus also done to other castings which are not under the same stress of high temperature and which ordinarily would not expand out of shape to such a great extent.

For the purposes of this specification we term this failure of such castings to return, after repeated expansions, to their original or true dimensions, as "growth". In other words, they eventually grow or increase in size, and suffer an undue permanent deformation. This "growth" continues with repeated expansions, with its destructive action, until the very body of the cast-iron begins to tear apart and cracks appear in the castings.

After these cracks are once started, deteriorating elements in the combustion of the fuel are able to penetrate into these cracks and help add

to the destructive action taking place. These cracks eventually enlarge to such an extent that finally a direct break will occur and a hole be gradually burned through the casting.

After careful investigations and study we have found that when chromium is introduced into cast-iron, it refines the grain of the casting, delays the breaking up of that constituent, or those constituents, which promote the general tensile strength of gray iron castings, and stops or substantially stops growth and cracking in the casting.

In our experiments and developments we have discovered that the above mentioned defects and disadvantages can be substantially eliminated by adding to the molten cast-iron from 1 to 1.5 percent of chromium, the molten cast-iron being raised, prior to the addition of the chromium, to a temperature somewhat higher than that used in customary gray iron practice, and the molten iron, after the addition of the chromium, being more quickly transferred to the mold and poured immediately to avoid undue cooling of the iron.

Among the objects of our invention are the overcoming of the disadvantages and the gaining of the advantages pointed out above.

A further object is the prevention of substantial growth in cast-iron parts subjected to considerable and frequent heating.

Another object is the prevention of substantial cracking in cast-iron parts subjected to considerable and frequent heating.

A still further object is the provision of novel steps in handling the cast-iron in melting it and adding chromium thereto in proper proportions.

A further object is the addition of the chromium to the molten cast-iron at the proper time and place, the heating of the iron to a higher temperature, and the quick handling of the molten iron after the chromium is added.

Another object is the production of a new iron alloy for the purposes stated.

Other objects, advantages and capabilities inherent in our invention will later more fully appear.

The growth or permanent substantial deformation of the usual cast-iron parts subjected to considerable heat causes considerable difficulty when it is necessary to replace an old permanently deformed part with a new part that is required to correctly interfit with another part that is likewise permanently deformed. The new part in such instances does not properly interfit with the old part because of the new part having the correct original dimensions while the original di-

mensions of the old part are greatly changed as a result of the permanent deformation or growth. An instance of this is found in cast-iron warm air furnaces and stoves which have been in use 5 for some time and in which it is found necessary to replace one of the parts, such as in the firepot, fire dome, grates, etc., these being the parts subjected to the most heat and consequent deformation. When such new part does not interfit with the cooperating old part it is generally necessary to have to also order another new part to take the place of the old part, thus involving additional delay as well as further expense.

15 By our present invention this delay and additional expense is avoided, thus affording the purchasing public the advantage of economy as well as saving in time. Many other instances than the specific parts of heating furnaces and stoves mentioned above could be cited, but these serve as 20 passing illustrations of the value to the general public of the present invention. With cast-iron parts made in accordance with the present invention such repairs or replacement will be necessary much less frequently, and even should they, in greater length of time, be needed the expense and delay would be very much less.

In the production of the alloy of the present invention we add chromium to the molten cast-iron, either in the cupola or preferably as it runs 30 from the cupola or other melting device, in an amount approximately between 1 to 2 percent. Among the compositions or mixtures of the cast-iron to which we have found it especially advantageous to add the chromium, and preferably 35 from 1 to 1.50 percent, is:—

|             |                       |
|-------------|-----------------------|
| Carbon      | 3.00 to 4.00 percent  |
| Silicon     | 2.25 to 2.75 percent  |
| Sulphur     | .05 percent and under |
| Phosphorous | .50 to .80 percent    |
| Manganese   | .50 to 1.00 percent   |

the balance being approximately pure iron. Materials of other and varying contents may be 45 similarly treated to advantage with a similar content of chromium. Where we add the chromium to the molten metal in the cupola, we prefer to have the chromium in the form of briquettes.

The chromium we preferably obtain in the form 50 of what is commercially called ferro chrome, which contains from 65 to 70 percent chromium, 3 to 4 percent silicon and 4 to 5 percent carbon. This ferro chrome is granular, the grains being preferably about one-twentieth of an inch and 55 smaller. The size of the grains may vary, the smaller the better, but the grains should be large enough to avoid undue blowing away by wind currents or the like.

We have found that a mixture of approximately 60 the following proportions is well adapted for the purposes of our invention:

|             |                        |
|-------------|------------------------|
| Carbon      | 3.00 to 4.00 percent   |
| Silicon     | 2.25 to 2.75 percent   |
| Sulphur     | .05 percent and under  |
| Phosphorous | .50 to .80 percent     |
| Manganese   | .50 to 1.00 percent    |
| Chromium    | 1.00 to 2.00 percent   |
| Pure iron   | 92.70 to 89.45 percent |

70 In the carrying out of our improved method for the production of our new alloy, the cast-iron, which is preferably a mixture of scrap and pig iron, is melted in a cupola or the like to a temperature somewhat higher than that employed in the usual gray iron practice. The

chromium is preferably added after the molten iron emerges from the tap hole in the breast of the cupola, the addition of the chromium occurring intermediate the tap hole and the receiving ladle. In our particular practice the molten iron 5 flows from the tap hole down an inclined stationary spout and into a tiltable spout that can be tilted to either side in order to conduct the flowing stream of molten iron into a receiving ladle on either side of the front of the cupola. 10

We have found it good practice to introduce the chromium into the flowing stream of molten iron at the point where the stream passes from the stationary spout of the cupola into the tilting spout for conducting it to the ladle. The 15 chromium may be in the form known commercially as ferro chrome. The desired amount of this ferro chrome may be placed in a container positioned just above the point of delivery of chromium to the molten iron, which container 20 may be open at the top and provided on its bottom with a downwardly extending spout of such size in cross-section as to deliver the ferro chrome into the molten stream of iron at such speed that the period of flow of the desired amount 25 of chromium will be from the time that about the first fifty pounds of molten iron is accumulated in say, for example, a one thousand pound ladle, up to shortly before the ladle is filled to its intended capacity. Just the intended amount 30 for the size of the ladle being used may be dumped into the container so that within the time just enumerated this amount will flow through the spout of the container and the container be emptied at the desired time prior to the filling of 35 the ladle; or, if desired, a greater amount of the ferro chrome may be placed in a container having a spout that will give a certain rate of flow, and the opening of the spout be opened and closed at the desired times, the amount of chromium added 40 being determined by the length of the time of flow.

Assuming the receiving ladle to hold one thousand pounds of molten iron, about fifty pounds of molten iron may be run into the bottom of the 45 ladle and the stream of ferro chrome then started and continued, as pointed out, up to shortly before the ladle is filled to its intended capacity, when the stream of chromium will either have stopped of its own accord if the container holds only the desired amount for one ladle full of iron, or the stream will be cut off at that time shortly before the ladle is filled to its intended capacity if the amount of chromium is being regulated by rate of flow. As the percentage of chromium in 55 the commercial ferro chrome runs about 70 percent chromium, we have found that about sixteen and one-half pounds of this commercial ferro chrome to one thousand pounds of molten iron can be satisfactorily used. This would give approximately eleven and fifty-five hundredths pounds (11.55 lbs.) of chromium to one thousand pounds of molten iron or, in other words, would add from approximately 1 to 2 percent of chromium to the iron. This exact proportion may be 60 somewhat varied but we find it to be satisfactory when the percentage of chromium runs somewhere between 1 to 2 percent.

While we have stated the exact point of the flowing stream of molten iron at which we prefer 70 to add the chromium, this point may be varied within reasonable limits. The chromium will be partially mixed with the stream of molten iron as it flows along the spout and into the ladle, which mixing will be completed in the ladle by 75

the ebullition or boiling action of the molten iron within the ladle.

As soon as the ladle is filled to its intended capacity with the mixture of molten iron and chromium, the transporting of the ladle to the mold or to such other ladle as the molten iron may be transferred to, and the pouring of the mold, is to be accomplished in a shorter time than is usual in the customary gray iron practice, as the addition of the chromium to the molten iron creates a tendency for it to solidify quicker than would such iron without chromium being added thereto.

No mechanical mixing is necessary as the action of the flowing stream of molten iron, together with the boiling action of the molten iron in the ladle, is sufficient to thoroughly mix the chromium with the molten iron.

Some of the articles made from the iron alloy and by the method disclosed herein are set forth and claimed in the copending application of William J. Doyle, Serial No. 41,283, filed September 19, 1935.

While the percentages of ingredients of the iron alloy given above may be varied, the limits stated herein are considered as giving satisfactory results.

Having now described our invention, we claim:—

30 1. The method of producing an iron alloy that will not suffer undue permanent growth or cracking from high heating, which consists in melting the iron in a cupola or the like at a higher temperature than customary in gray iron practice, flowing the molten iron in a stream from the cupola to a ladle until a small amount of molten iron is accumulated in the ladle, then flowing a stream of granular ferro chrome of approximately 70 percent chromium content into the 40 flowing stream of molten iron intermediate the cupola and the ladle, and stopping the flow of the stream of ferro chrome shortly before the ladle

is filled to its intended capacity, and transporting the molten iron to and pouring it into a mold more quickly than is customary in gray iron practice.

2. That step in the method of producing a 5 cast-iron alloy that will not suffer undue permanent growth or cracking from heating, which consists in adding from 1 to 1.50 percent of chromium to the flowing stream of molten iron as it flows from a cupola or the like, the chromium 10 being granular and added in a flowing stream to the flowing stream of molten iron at a point intermediate the ladle and the cupola tap hole.

3. The method of producing an iron alloy that will not suffer undue substantial growth, deformation or cracking from heating, which consists in melting cast-iron in a cupola, or the like, at a temperature higher than that used in customary gray iron practice, measuring out such quantity of ferro chrome in granular form of approximately 70 percent chromium content that will add from between 1 to 2 percent of chromium to the molten iron when the ladle is filled to its intended capacity, placing said ferro chrome in a container having a spout and supported above 20 the cupola spout between the tap hole and the ladle, flowing the molten iron in a stream from the cupola to a ladle until a small amount of molten iron is accumulated in the ladle, then causing the granular ferro chrome to flow in a 25 stream from said container into the stream of molten iron at a point between the tap hole and the ladle, regulating the flow of ferro chrome so that the required amount will have completed its 30 flow into the flowing stream of molten iron shortly before the ladle is filled to its intended capacity, and transporting the molten iron to and pouring it into a mold more quickly than is customary in gray iron practice.

40  
WILLIAM J. DOYLE.  
JUSTUS J. WOLLENHAUPT.